

Sept. 14, 1926.

J. R. BROWN ET AL

1,599,608

ELECTROPLATED ARTICLE AND METHOD OF MAKING SAME

Original Filed Feb. 11, 1922



Fig. 1



Fig. 2



Fig. 3



Fig. 4



Fig. 5

INVENTORS

Tolles Rowland Brown and  
BY John C. Mullinix.

Day, Oberlin & Day  
ATTORNEYS.

Patented Sept. 14, 1926.

1,599,608

# UNITED STATES PATENT OFFICE.

JOHN ROWLAND BROWN AND JOHN C. MULLINNIX, OF CLEVELAND, OHIO, ASSIGNEES  
TO THE RELIANCE GAUGE COLUMN COMPANY, OF CLEVELAND, OHIO, A CORPOR-  
ATION OF OHIO.

## ELECTROPLATED ARTICLE AND METHOD OF MAKING SAME.

Application filed February 11, 1922, Serial No. 535,951. Renewed June 21, 1924.

The present improved method of making electro-plated articles has been developed in connection with the manufacture of hollow articles and particularly floats of the kind used in steam traps, water columns, etc., the object being to make a float composed of an internal hollow foundation and an external seamless metallic shell electro-deposited thereon, instead of spinning the float from sheet metal in hemispheres and then lapping together and brazing the two sections at the joint, as is the current practice in manufacturing such floats. The present improvements, however, are not limited to the manufacture of such floats, or even to hollow articles, but at least in certain phases will be found of utility in electro-plating solid forms composed of various materials, as for example in the manufacture of statuary, vases and other art objects.

Where non-metallic articles are to be electro-plated it is, of course, necessary first to coat the same with finely powdered graphite or with some equivalent material that will render the surface a conductor for electricity. For many purposes the present practice is to use in place of such graphite, bronze or copper powder (copper "schliff"), and one object of the present invention accordingly is to provide an improved method for attaching a coating of such metallic powder in uniformly distributed condition over the surface of the article to be plated. Resulting from such method of attachment an article having certain novel characteristics is produced. To the accomplishment of the foregoing and related ends, the invention then consists of the steps and means hereinafter fully described and particularly pointed out in the claims, the annexed drawing and the following description setting forth in detail certain steps and means embodying the invention, such disclosed steps and means constituting, however, but one of various ways in which the principle of the invention may be used.

In said annexed drawing:

Fig. 1 is a perspective view of an internal hollow foundation or core suitable for use in the manufacture of a hollow spherical float, in accordance with our present improved method; Fig. 2 is a central section, on a somewhat larger scale, through

such foundation, showing as assembled therewith the spud whereby the float when completed may be connected with suitable operating mechanism; Fig. 3 is a sectional view showing the foundation after it has received a coating of celluloid or celluloid-like material that forms an intermediate layer of the completed article; Fig. 4 is a view similar to Fig. 3, but showing the article in a subsequent stage of its manufacture; and Fig. 5 is a view likewise similar to Fig. 3, but showing the completed article, i. e., after the outer metal coat has been electro-deposited on the foundation or core.

The core or foundation 1, while shown in the drawing as of approximately spherical form, may of course take on any shape required by the exigencies of the use to which the completed float is to be put. For that matter, as pointed out above, our improved process is not limited to the fabrication of floats but is applicable to the making of various articles, either hollow or solid, where a non-metallic foundation is to be coated with a thin layer of metal. The spud 2, shown as attached to the core in Fig. 2, accordingly is a feature of incidental interest only and may not be required at all where the article to be made requires no external attaching means, the particular spud shown forming the subject-matter of a separate application filed by John Rowland Brown, one of the present inventors, viz., Ser. No. 505,524, filed October 5, 1921.

Where the device is intended for use as a float, the core 1 is preferably molded from pulp material, as for example, wood pulp or papier-mâché, and is characterized by having its exterior surface closely and more or less uniformly dotted with small rounded protuberances 3, this particular type of core likewise forming the subject-matter of a separate application filed by the present inventors February 8, 1922, Ser. No. 535,037. So far as the present improved process is concerned, such surface may be entirely smooth, such process primarily relating, as previously indicated, to the preparation of the surface, whatever its character, for the electro-deposition of the metallic coating.

According to the present process, assuming where a spud or like element is to be

attached to the foundation that the same has been suitably cemented in place, the foundation or core is then given a coating of acid-resisting lacquer capable of receiving and holding a coating of bronze or copper powder in the fashion now to be described. As a lacquer admirably suited for the purpose we employ a cellulose ester, as the nitrate or acetate, dissolved in one or more of the known solvents therefor. For example, pyroxylin or celluloid thus dissolved in a suitable liquid vehicle and capable of hardening when subjected to evaporation or other treatment will serve as a satisfactory lacquer for the purpose. After the first coating of such lacquer has been applied, the surface, particularly where the core is made of molded pulp material, is sandpapered or otherwise polished so as to remove any tiny projecting strands of the base material. Thereupon one or more additional coats of the same or a similar lacquer are applied, the coating being conveniently accomplished by simply dipping the core or foundation in a bath of the lacquer maintained in proper fluid condition. Thus there is built up, closely surrounding the core or foundation, a shell of pyroxylin, cellulose or equivalent cellulosic derivative, and it is upon this shell that the final coat of metal is deposited.

It is necessary first, however, to coat such intermediate shell with electro-conductive material, as previously explained. To this end such material, for example, the bronze or copper powder hereinbefore referred to, is thoroughly mixed in a liquid vehicle consisting of a solvent for the celluloid or equivalent layer, for example, amyl acetate, chlorhydrin or like known solvent. Preferably a small quantity of the pyroxylin or other cellulosic derivative is also included in such mixture, the latter being left sufficiently fluid to permit it to be applied to the core or foundation by spraying with an air brush or like device. A thin uniform coating of such mixture is applied with the result that the solvent ingredient will soften the exterior surface of the previously applied layer or coat sufficiently to render the same "tacky," thereby causing the fine metal particles to firmly adhere; but the evaporation of the solvent ingredient leaves such particles otherwise exposed, so that they are not coated with the pyroxylin and so prevented from subserving their proper function as a conductor for the electric current.

The articles thus prepared are now ready to be immersed in an electrolytic bath and a coating of copper or other metal is thereupon deposited on the surface of the article in the usual way.

Preliminarily to the application of the first coat of lacquer, we find it desirable to heat the core, where the latter is of the hollow

type illustrated and required for use in the case of floats or similar articles, the point to which such heating is carried being determined by the temperature which the material composing the core will stand without injury. The result will of course be the expansion of the air or other gas within the core so that when the latter is subsequently immersed in a bath of lacquer, which is maintained at a lower temperature, preferably as cold as it can be conveniently maintained without rendering it too stiff, the air within the core will contract and so create a suction effect that will tend to cause the lacquer to penetrate the core rather than just cling to the surface. Indeed where the relative temperatures of the core and lacquer are reversed, there is a tendency for the air upon expansion during the dipping operation to escape through the core and form bubbles under the coating of lacquer.

Other forms may be employed embodying the features of our invention instead of the one here explained, change being made in the form or construction, provided the elements stated by any of the following claims or the equivalent of such stated elements be employed, whether produced by our preferred method or by others embodying steps equivalent to those stated in the following claims.

We therefore particularly point out and distinctly claim as our invention:

1. In a method of electroplating a non-metallic article, the steps which consist in first coating such article with a cellulose derivative on the order of celluloid, then applying a coating of electro-conductive material, and thereupon electrolytically depositing the desired metal.

2. In a method of electroplating a non-metallic article, the steps which consist in first coating such article with a cellulose derivative on the order of celluloid, then applying a coating of electro-conductive material intermixed with a volatile solvent for such derivative as a vehicle, evaporating off such solvent, and thereupon electrolytically depositing the desired metal.

3. In a method of electroplating a non-metallic article, the steps which consist in first repeatedly dipping such article in a solution of a cellulose derivative on the order of celluloid and evaporating off the solvent until a substantial layer of such derivative is obtained, then spraying a coating of electro-conductive material intermixed with a volatile solvent for such derivative as a vehicle, evaporating off such solvent, and thereupon electrolytically depositing the desired metal.

4. In a method of electroplating a non-metallic article, the steps which consist in first repeatedly dipping such article in a

9. A hollow float or like article comprising a core molded from pulp material, a coating of celluloid applied to such core, and an electro-deposited coating of desired metal 55 surrounding such first coating.
10. An electroplating base, which comprises a hollow core of pulp material having a coating of a cellulosic derivative on the order of celluloid. 60
11. An electroplating base, which comprises a hollow core of pulp material, the exterior surface being covered with closely spaced small protuberances and having a coating of cellulosic derivative on the order 65 of celluloid.
12. In a method of coating a hollow article molded from pulp material so as to render the same non-permeable to air, the step which consists in dipping such article 70 in a solution of a cellulosic derivative on the order of celluloid, the temperature of such article being higher than that of such solution.
13. In a method of coating a hollow article 75 molded from pulp material so as to render the same non-permeable to air the steps which consist in dipping such article in a solution of a cellulosic derivative on the order of celluloid, the temperature of 80 such article being higher than that of such solution, evaporating off the solvent so as to leave a coating of such derivative, polishing the article thus coated, similarly applying one or more additional coatings of such derivative until a substantial layer thereof is obtained, 85 then spraying a coating of electro-conductive material intermixed with a volatile solvent for such derivative as a vehicle, evaporating off such solvent, and thereupon electrolytically depositing the desired metal.
14. In a method of coating a hollow article 90 molded from pulp material so as to render the same non-permeable to air, the steps which consist in dipping such article in a solution of a cellulosic derivative on the order of celluloid, polishing the article thus coated, and thereupon applying one or 95 more additional coatings of such derivative until a substantial layer thereof is obtained.
15. In a method of electroplating a hollow air-permeable article, the steps which consist in dipping same in a bath of acid-resisting lacquer, the interior of such article being sealed with air or other gaseous medium 10 therein and the temperature of such article being higher than that of such bath, removing the article from such bath, whereupon the contraction of the air or other gaseous medium therein due to cooling will create 15 a suction effect, then applying to the article a coating of electro-conductive material, and thereupon electrolytically depositing the desired metal.
16. In a method of electroplating a hollow article 20 molded from pulp material, the steps which consist in dipping same in a solution of a cellulose derivative on the order of celluloid, the temperature of such article being higher than that of such solution, evaporating off the solvent so as to leave a coating of such derivative, polishing the article thus coated, similarly applying one or more additional coatings of such derivative until a substantial layer thereof is obtained, then spraying a coating of electro-conductive material intermixed with a volatile solvent for such derivative as a vehicle, evaporating off such solvent, and thereupon electrolytically depositing the desired metal.
17. An electroplated article comprising a core of non-metallic material other than celluloid, a coating of a cellulose derivative on the order of celluloid applied to such core, and an electro-deposited coating of desired metal 25 surrounding such first coating.
18. An electroplated article comprising a core 30 molded from pulp material, a coating of a cellulose derivative on the order of celluloid applied to such core, and an electro-deposited coating of desired metal surrounding such first coating.

Signed by us, this 7th day of February, 1922.

JOHN ROWLAND BROWN.  
JOHN C. MULLINNIX.